

# United States Patent Office

3,232,763  
Patented Feb. 1, 1966

## 1

3,232,763

### GELATIN COMPOSITIONS CONTAINING A BISISOMALEIMIDE HARDENER

Donald M. Burness and Burton D. Wilson, Rochester, N.Y., assignors to Eastman Kodak Company, Rochester, N.Y., a corporation of New Jersey  
No Drawing. Filed Mar. 14, 1963, Ser. No. 265,043  
5 Claims. (Cl. 96—111)

This invention relates to gelatin coating compositions and layers prepared therefrom composed of gelatin and as a hardener therein an alkylene bisismaleimide, the alkylene being of 4 to 10 carbon atoms.

Various bismaleimides have been proposed as gelatin hardeners as for instance in U.S. Patent 2,992,109 of C. F. H. Allen and Belgian Patent 579,914 of Gevaert Photo-Products. It has been noted that incorporation of hexamethylene bismaleimide in a gelatin composition produces only a slight increase, if at all, in the melting points of the gelatin layers obtained therefrom.

10

15

20

## 2

### Example 1

The procedure described by Cotter, Sauers and Whelan, Journal of Organic Chemistry, volume 26, page 10 (1961), was followed using commercial dicyclohexylcarbodiimide. The product obtained was in the form of colorless crystals in 52% yield which product had a melting point of 96.5–97.5° C. Samples of this product, hexamethylene bisismaleimide, were added to separate portions of a high speed gelatin-silver bromoiodide emulsion, which had been panchromatically sensitized with a cyanine dye, in the proportions indicated in the table. As a comparison samples of the emulsion without hardener added and with hexamethylene bismaleimide in corresponding proportion were taken. Each of these emulsion samples was coated out onto cellulose acetate film support at a coverage of 432 mg. of silver and 980 mg. of gelatin per square foot. A sample of each film coating was exposed on an Eastman 1B sensitometer, processed for 5 minutes in Kodak DK-50 developer, fixed, washed and dried with the following results:

| Compound Name                           | Conc.,<br>g./100<br>g. of gel | Rel.<br>Speed | γ    | Fog  | Percent<br>Swell <sup>1</sup> | Ret.,<br>° F. <sup>2</sup> | M.P.,<br>° F. <sup>3</sup> |
|-----------------------------------------|-------------------------------|---------------|------|------|-------------------------------|----------------------------|----------------------------|
| Control                                 | —                             | 100           | 1.32 | 0.14 | 716                           | 84                         | 88                         |
| N,N'-Hexamethylene-bis-<br>maleimide    | 0.6                           | 85            | 1.37 | 0.12 | 477                           | 82                         | 91                         |
| Do                                      | 1.2                           | 89            | 1.46 | 0.12 | 469                           | 77                         | 92                         |
| N,N'-Hexamethylene-bis-<br>isomaleimide | 0.6                           | 74            | 1.33 | 0.11 | 433                           | 94                         | 123                        |
| Do                                      | 1.2                           | 54            | 1.30 | 0.10 | 329                           | None                       | >212                       |

<sup>1</sup> Vertical swell in water without processing.

<sup>2</sup> Reticulation, ° F.

<sup>3</sup> Melting Point, ° F.

One object of our invention is to provide a hardener which produces a large increase in melting point and reduction of swell in gelatin layers. Another object of our invention is to provide compositions useful for photographic purposes composed of gelatin and an alkylene bisismaleimide. Other objects of our invention will appear herein.

We have found that compounds of the following structure when incorporated in gelatin compositions effectively harden the gelatin layers therefrom as evidenced by their greatly increased melting points and resistance to swelling by water:



where  $n$  is an integer of 4 to 10.

We have found that these compounds of our invention when incorporated in gelatin layers at a concentration as little as 0.5% of the gelatin will effectively harden the gelatin so as to increase the melting point and resistance to swelling by water of layers prepared therefrom. We have found that these hardeners have no detrimental effect on the photographic properties of products in whose preparation they are used.

The following examples illustrate the use of compounds in accordance with the invention for gelatin hardening comparing same with the effectiveness of bismaleimide hardeners.

35

40

The melting points were determined by placing the samples in water and increasing the temperature of the water until the emulsion coating disintegrated. The temperature at this point designated the melting point of the gelatin containing layer.

### Example 2

A slurry of 51.2 grams of N,N'-tetramethylene-bis-maleamic acid in 500 ml. of dichloromethane was stirred vigorously while a solution of 82.5 grams of commercial dicyclohexylcarbodiimide in 75 ml. of dichloromethane was added dropwise over a period of 50 minutes. The mixture was stirred for 24 hours, then cooled and the solids were removed by filtration. The crude residue was extracted with hot benzene, filtered and evaporated to dryness. The residue was slurried with cold ether and filtered. The crude, colorless crystalline solid was recrystallized with benzene-ether to give N,N'-tetramethylenebisismaleimide having a melting point of 146.5 to 148.5° C.

The tetramethylene bisismaleimide prepared in Example 2 was added to separate portions of high-speed silver bromoiodide emulsion which had been panchromatically sensitized with a cyanine dye, in the proportions indicated in the table. A sample of the emulsion without hardener was also taken. Each emulsion sample was coated onto a cellulose acetate film support at a coverage of 459 mg. of silver and 1040 mg. of gelatin per square foot. A sample of each film coating was exposed on an Eastman 1B sensitometer, processed for five min-

55

60

65

utes in Kodak DK-50 developer, fixed, washed and dried with the following results:

2. A composition comprising gelatin containing therein hexamethylene bisisomaleimide.

| Compound Name                           | Cone.,<br>g./100<br>g. of gel | Rel.<br>Speed | $\gamma$ | Fog | Swell <sup>1</sup> | Ret.,<br>°F. | M.P.,<br>°F. |
|-----------------------------------------|-------------------------------|---------------|----------|-----|--------------------|--------------|--------------|
| Control                                 | -----                         | 100           | 1.02     | .17 | 730                | 74           | 85           |
| N,N'-Tetramethylenebisiso-<br>maleimide | 3                             | 76            | 1.22     | .12 | 320                | None         | >212         |
| Do                                      | 6                             | 59            | 1.17     | .10 | 280                | None         | >212         |

<sup>1</sup> Taken after developing, fixing and washing.

The hardeners in accordance with our invention are useful for incorporation in gelatin coating compositions generally, not only for use as hardeners for gelatin silver halide photographic emulsions but also for use in gelatin compositions employed for antihalation layers, baryta layers, antistatic layers, over-coatings or any other instance where a gelatin layer is used in preparing a photographic product.

We claim:

1. A gelatin-silver halide photographic emulsion containing therein a hardening amount of



*n* being an integer of 4 to 10.

3. A composition comprising gelatin containing therein tetramethylene bisisomaleimide.

4. A gelatin-silver halide photographic emulsion containing hexamethylene bisisomaleimide.

5. A gelatin-silver halide photographic emulsion containing therein tetramethylene bisisomaleimide.

20 References Cited by the Examiner

UNITED STATES PATENTS

|           |         |                    |         |
|-----------|---------|--------------------|---------|
| 2,726,162 | 12/1955 | Allen et al.       | 106—125 |
| 2,899,327 | 8/1959  | Christopher et al. | 106—125 |
| 2,992,109 | 7/1961  | Allen              | 96—111  |
| 2,994,611 | 8/1961  | Heyna et al.       | 96—111  |

25 OTHER REFERENCES

Chemical Abstracts, vol. 55 (1961), pp. 19782 to 19784.

NORMAN G. TORCHIN, Primary Examiner.